

Dec. 19, 1933.

E. MAHLE

1,940,629

PISTON ALLOY

Filed Oct. 30, 1931

*Fig. 1.*



*Fig. 2.*



*Fig. 3.*



*Fig. 4.*



*Ernst Mahle*  
INVENTOR.

BY

*Hausfeld & Warland*  
ATTORNEYS.

## UNITED STATES PATENT OFFICE

1,940,629

## PISTON ALLOY

Ernst Mahle, Stuttgart, Germany, assignor to  
Elektronmetall G. m. b. H., Cannstatt-Stutt-  
gart, Germany

Application October 30, 1931, Serial No. 572,071,  
and in Germany November 1, 1930

6 Claims. (Cl. 309—14)

This invention relates to improvements in pistons for internal-combustion engines.

More particularly the invention relates to the employment of alloys—some of which are already known—of copper and beryllium (beryllium bronzes) as structural material for the pistons of internal combustion engines.

During recent years, light metal alloys have come more and more into favour as piston materials, in place of the grey cast iron at one time exclusively used for that purpose. It has, however, been found that the low hardness of these light-metal alloys at high temperatures constitutes a defect which must be set off against the numerous favourable properties which have substantially contributed to the extended use of said alloys. This defect becomes extremely serious in the piston-ring grooves, inasmuch as the grooves which are exposed to the greatest thermal action, namely near the head, are unable to offer any prolonged resistance to the impact of the piston rings, but become battered at the prevalent high temperatures, so that the pistons are no longer accurately guided, and, in some events, are even rendered useless.

Attempts to improve the high-temperature hardness of the light metals to a substantial extent by incorporating new alloying components, have failed.

It has now been ascertained in accordance with the invention, that certain beryllium bronzes, which must be classed among the heavy metals, exhibit a quite unusual high-temperature hardness which seems to render them particularly suitable as structural material for pistons, at least for the ring portions of same. In such case the actual body of the piston can still be made of light metal, that portion of the end, in which the piston rings are fitted, being rolled-in or integrally cast-in an annular shell. However, the entire end of the piston, including the portion carrying the piston rings, may also consist of beryllium bronze.

As compared with the suggestions for improving the high-temperature hardness of the ring portion by constructing it of grey cast iron and suitably connecting it with the other, light-metal, portion of the piston, the construction of the ring portion of beryllium bronze, in accordance with the invention, offers the advantage that the thermal expansion of these alloys approximates far more closely to that of the light-metal alloys, so that many constructional disadvantages arising from the necessity of ob-

taining secure connection between the cast iron and light-metal parts of the piston are obviated. A further advantage over that arrangement consists also in that the heat conductivity of the copper-beryllium alloys is superior to that of grey cast iron, so that the good conductivity constituting one of the main advantages of the light-metal alloys is not impaired, in the present case, to the same extent as when cast iron is used for the ring portion.

In view of the relatively high thermal expansion of the beryllium bronzes, it is advisable, where stress is laid on the noiseless running of the engine, to employ copper-beryllium alloys solely for that portion of the piston that carries the rings, and to make the skirt for which high-temperature hardness and heat conductivity are of minor importance, of grey cast iron or steel plate. In this manner a method of construction is attained in which a head of light metal is surrounded by a beryllium-bronze shell, provided with the piston-ring grooves and carrying a skirt portion of iron, the several structural components being connected together in known manner, but without the previously encountered difficulties, since the differences in the coefficients of thermal expansion of the successive materials merge gradually into one another.

In order more clearly to understand the invention, reference is made to the accompanying drawing which illustrates by way of example, two embodiments of pistons constructed in accordance therewith and in which:

Fig. 1 is a vertical section taken through the gudgeon pin bosses, of one embodiment;

Fig. 2 is a vertical section taken at right angles to Fig. 1;

Fig. 3 is a plan section along the line A—B of Fig. 1; and

Fig. 4 is a vertical section taken through the gudgeon pin bosses, of a second embodiment.

In both embodiments the piston head 1 is made of light metal, in order to reduce the moving mass, whilst a portion 2, carrying the piston rings and secured to the piston head in any suitable known manner (such as by shrinking-on or integral casting) is made of a copper-beryllium alloy of high Brinell hardness at high temperatures and good heat conductivity. The piston skirt 3 is of iron, in order to obtain high resistance to abrasion and low heat expansion in this part of the piston (which is subjected to heavy sliding friction), and is attached to the piston head by screws or rivets 4 in the embodiment shown in Figs. 1 to 3 or by ribs 5, integrally

cast with the shell 2 in the embodiment shown in Fig. 4.

In other cases, (such as Diesel engines) where high thermal expansion in the piston skirt is a matter of no importance, the skirt also may consist of beryllium bronze, it being advisable to incorporate a certain amount of manganese in the alloy, in order to increase the resistance to abrasion.

10 Materials that have been found particularly suitable for the purpose of the present invention, are binary alloys of copper with up to 5 percent (preferably about 2.5 percent) of beryllium, which still exhibit a high-temperature hardness of about 200° Brinell at 350° C. Increased resistance to abrasion, with the same high-temperature hardness, is obtained by the employment of certain alloys of copper with minor quantities of beryllium and manganese, which 15 may be subjected to heat treatment with a view of further improving their hardness at lower temperatures. Thus, an alloy containing about 1.5 percent of beryllium and about 3 percent of manganese, the balance being copper, has a 20 hardness of about 200° Brinell at 350° C. in the untreated as well as the heat-treated form. At ordinary temperatures, however, the hardness of the untreated alloy amounts to only about 150° Brinell, whereas, after a heat treatment comprising heating the alloy to about 750° C. and then quenching, the hardness at ordinary temperatures rises up to about 300° Brinell.

I claim:

1. A piston for internal combustion engines having a ring-bearing portion composed of a beryllium bronze, having copper as its main constituent and containing between about 1 and about 5 percent of beryllium, and having the portion contacting the ring-bearing portion composed of a different metal having a coefficient of expansion approximating that of the beryllium bronze.

2. A piston for internal combustion engines having a ring-bearing portion composed of a beryllium bronze, having copper as its main constituent and containing between about 1 and about 5 percent of beryllium, and about 3 per-

cent of manganese, and having the portion contacting the ring-bearing portion composed of a different metal having a coefficient of expansion approximating that of the beryllium bronze.

3. A piston for internal combustion engines 80 having a ring-bearing portion composed of a beryllium bronze, the constituents of which are about 1 to about 5 percent of beryllium, about 3 percent of manganese, the remainder being copper, and having the portion contacting the ring-bearing portion composed of a different metal having a coefficient of expansion approximating that of the beryllium bronze.

4. A piston for internal combustion engines 90 having a ring-bearing portion composed of a beryllium bronze, the constituents of which are 1.5 percent of beryllium, 3 percent of manganese, and 95.5 percent of copper, and having the portion contacting the ring-bearing portion composed of a different metal having a coefficient of expansion approximating that of the beryllium bronze.

5. A piston for internal combustion engines comprising a piston-head of light metal, an annular shell composed of a beryllium bronze having copper as its major constituent and containing between about 1 and about 5 percent of beryllium and having a coefficient of expansion approximating that of said light metal surrounding said piston head, grooves adapted to receive 100 piston rings in said annular shell and a skirt portion substantially consisting of iron connected with said annular shell.

6. A piston for internal combustion engines comprising a piston head of light metal, an annular shell, composed of a beryllium bronze, the constituents of which are between about 1 and about 5 percent of beryllium, 3 percent of manganese, and the remainder of copper, and the coefficient of expansion of which approximates 110 that of said light metal, surrounding said piston head, grooves adapted to receive piston rings in 115 said annular shell and a skirt portion substantially consisting of iron connected with said annular shell.

120 ERNST MAHLE.

50

125

55

130

60

135

65

140

70

145

75

150